

[54] **FUNCTIONAL FLUIDS CONTAINING AMMONIUM SALTS OF PHOSPHORUS ACIDS**

[75] Inventors: **Theodore A. Marolewski**, New City; **Fred Jaffe**, Ossining, both of N.Y.

[73] Assignee: **Stauffer Chemical Company**, Westport, Conn.

[\*] Notice: The portion of the term of this patent subsequent to Mar. 2, 1993, has been disclaimed.

[21] Appl. No.: **658,428**

[22] Filed: **Feb. 17, 1976**

#### Related U.S. Application Data

[63] Continuation-in-part of Ser. No. 441,698, Feb. 11, 1974, abandoned.

[51] Int. Cl.<sup>3</sup> ..... **C10M 3/40**

[52] U.S. Cl. ..... **252/78.5**

[58] Field of Search ..... **252/78, 49.8, 49.9, 252/78.5**

#### [56] References Cited

##### U.S. PATENT DOCUMENTS

|           |         |                        |          |
|-----------|---------|------------------------|----------|
| 3,311,560 | 3/1967  | Hotten .....           | 252/78 X |
| 3,707,501 | 12/1972 | Gentit et al. ....     | 252/78   |
| 3,790,487 | 2/1974  | Burrous .....          | 252/78   |
| 3,793,199 | 2/1974  | Schlicht .....         | 252/78 X |
| 3,941,708 | 3/1976  | Gentit et al. ....     | 252/78   |
| 3,956,154 | 5/1976  | Marolewski et al. .... | 252/78   |

#### OTHER PUBLICATIONS

Preprint of Symposium on Deposit, Wear and Emission Control by Lubricants and Fuel Additives, Division of Petroleum Chemistry, Inc., Amer. Chem. Soc., N.Y.C. Meeting, Sep. 7-12, 1969.

Primary Examiner—Harris A. Pitlick  
Attorney, Agent, or Firm—Roger S. Benjamin

#### [57] ABSTRACT

A composition and method for inhibiting damage in a functional fluid by incorporating therein a damage inhibiting amount of an ammonium salt of a phosphorus acid in accordance with the formula:



wherein R, R', R'', R''' can be the same or different and wherein R and R' can be conjoint and contain oxygen, nitrogen, and mixtures thereof; and represent alkyl, aralkyl, and alkenyl groups containing from 1 to about 30 carbon atoms, X represents oxygen or sulfur, Y' and Y'' represent lower alkoxy, lower thioalkoxy, alkenyloxy, thioalkenyloxy, lower alkyl, carboalkoxyalkyl, phenyl lower alkyl, thiophenoxy, aryloxy, alkaryloxy, aralkoxy and lower alkylthiophenoxy, Z represents oxygen or sulfur, and m equals 1 or 2.

6 Claims, 1 Drawing Figure

#### CONTAMINATION OF PHOSPHATE ESTER FLUID WITH CHLORINATED SOLVENTS



## CONTAMINATION OF PHOSPHATE ESTER FLUID WITH CHLORINATED SOLVENTS



## FUNCTIONAL FLUIDS CONTAINING AMMONIUM SALTS OF PHOSPHORUS ACIDS

This is a continuation-in-part of application Ser. No. 5  
441,698, now abandoned.

### BACKGROUND OF THE INVENTION

This invention relates to functional fluid compositions having the ability to inhibit and control damage to mechanical members in contact with these fluid compositions. 10

A wide variety of functional fluids are known and utilized for many applications. Functional fluids have been used as electronic coolants, atomic reactor coolants, diffusion pump fluids, lubricants, damping fluids, bases for grease, power transmission and hydraulic fluids, heat transfer fluids, heat pump fluids, refrigeration equipment fluids and as filter mediums for air conditioning systems. 15

In many of the functional fluid compositions used for the above purposes there have been reports of damage to the fluid during use and to mechanical members, especially metallic members in contact with the fluid, as evidenced by a loss of weight of such members, due to 25 the wearing away of metallic parts. Damage has been reported in aircraft hydraulic systems, gas turbine bearings, jet turbine control systems, steam turbine bearings, steam turbine control systems, electrohydraulic control systems and aerospace control equipment. Damage has also been observed on such materials as glass, Teflon, Mylar, Plexiglass and members constructed from other non-metallic materials. 30

In those instances where functional fluids are used in the hydraulic systems of aircraft and aerospace systems, such systems impose stringent requirements on the hydraulic fluid. Not only must these hydraulic fluids meet stringent use requirements but they must also satisfy 35 FAA and other government requirements for fire resistance. Additionally, the hydraulic fluid must be capable of performing in the hydraulic system over an extended period of time without causing significant damage or functional impairment to the various conduits, valves, pumps, and the like, through which the fluid flows in the course of such use. 40

Damage caused by functional fluids contacting valves and other members has been attributed to the wearing away or erosion of the environment in contact with the functional fluid in a hydraulic system. Among the many undesirable results caused by such damage is a marked decrease in strength of the structural mechanical parts in the hydraulic system, such as pumps and valves, along with an alteration of the geometry of these parts. Such changes in the case of pumps can cause a decrease in pumping efficiency, and in the case of 50 valves can cause faulty operations, excessive leakage and even hazardous conditions. 55

This damage necessitates costly and time consuming premature overhaul of mechanical parts. Additionally, metal removed from component metallic mechanical parts in contact with the functional fluid contaminates the fluids, causes filter clogging and excessive filter replacement, and requires premature draining and replacement of the fluid in the system. The metal contamination can also cause a change in physical and chemical 60 properties of the functional fluids. 65

Metal contaminants can also reduce the oxidative stability of a fluid, thereby adversely affecting fluid

performance. In addition, metal contamination of the fluid can manifest itself in numerous other ways, including viscosity change, increased acid number, formation of precipitates, decrease in chemical stability and discoloration.

Another problem in the industry is the unavoidable contamination of aircraft and electrohydraulic control systems with chlorinated solvents used to clean the systems and components. A detailed discussion of this problem appears in *Vickers 22nd Fluid Power Conference Report*, Oct. 30, 1972, Section 4, Pages 25-29. Contamination by chlorinated solvents decreases the service life of functional fluids and accelerates damage, causing excessive internal leakage in hydraulic systems to a point of malfunction. No additive heretofore known has satisfactorily overcome the problems associated with chlorinated solvent contamination of functional fluids. 10

In the past, there have been reports of damage to valves and other metallic members which contact phosphate ester fluids. U.S. Pat. No. 2,470,792 proposes to 20 overcome this damage problem by the inclusion of a small percentage of water in an aircraft hydraulic system. Unfortunately, while the presence of a small percentage of water reduces certain types of damage when incorporated in some phosphate ester hydraulic fluids, the presence of water can have a corrosive effect as well as an undesirable effect on the stability of the fluid.

U.S. Pat. No. 3,707,501 discloses the use of phosphonium compounds to inhibit erosion damage to the metallic environment containing hydraulic fluids. However, the lubricant compositions require relatively high concentrations of phosphonium compounds, which are very expensive. In addition, the phosphonium compounds may contribute to the destabilization of the functional fluid. 25

U.S. Pat. No. 3,679,587 discloses alkali salts of perfluorinated alkyl sulfonic acids as erosion inhibitors. However, since these compositions are ash containing materials, high temperature operation could lead to the formation of particulate matter in a hydraulic system. 30

### SUMMARY OF THE INVENTION

In accordance with the present invention, a functional fluid has been discovered which exhibits enhanced low erosion, shear, oxidative and thermal stability, and fire resistance characteristics, and is particularly suitable for aircraft hydraulic applications. This invention comprises the incorporation of a minor percentage of certain ammonium salts of phosphorus acids into various base stocks compositions so as to produce a functional fluid capable of inhibiting damage to the metal environment containing the functional fluid. 45

### DETAILED DESCRIPTION OF THE INVENTION

The ammonium salts of the phosphorus acids which are useful for incorporation in functional fluids in accordance with the present invention are represented by the following formula and description:



wherein R, R', R'', and R''' can be the same or different and wherein R and R' can be conjoint and contain oxy-

gen, nitrogen, and mixtures thereof; and represent alkyl, aralkyl, and alkenyl groups containing from 1 to about 30 carbon atoms, X represents oxygen or sulfur, Y' and Y'' represent lower alkoxy, lower thioalkoxy, alkenyloxy, thioalkenyloxy, lower alkyl, carboalkoxyalkyl, phenyl lower alkyl, thiophenoxy, aryloxy, alkaryloxy, aralkoxy and lower alkylthiophenoxy, Z represents oxygen or sulfur, and m equals 1 or 2. In a preferred embodiment, m=1.

An alternative embodiment involves the ammonium ions attached to the phosphorus anion via an alkylene or arylene group. This forms a zwitterion wherein the ions are connected, generally by a carbon or carbon and oxygen chain, as for example:



wherein R, R' and R''' are as above and R'' can be any divalent connecting unit such as  $CH_2$ , and x can vary from 1 to 10. Representative of the above is:



The following is a listing of typical ammonium salts of phosphorus acids tabulated according to the respective ammonium ions and phosphorus ester anions:

| Ammonium Ions                                           | Phosphorus Ester Anions                |
|---------------------------------------------------------|----------------------------------------|
| Dodecyl trimethyl ammonium                              | Diphenyl phosphate                     |
| Hexadecyl trimethyl ammonium                            | Phenyl phosphate<br>(bis-amine salt)   |
| Octadecyl trimethyl ammonium                            | Dimethyl phosphate                     |
| Tridecyl trimethyl ammonium                             | Methyl phosphate<br>(bis-amine salt)   |
| Decyl trimethyl ammonium                                | Methyl methylphosphonate               |
| Didodecyl dimethyl ammonium                             | Methylphosphonate<br>(bis-amine salt)  |
| Dimethyl propyl dodecyl ammonium                        | Diethyl phosphate                      |
| Diocetyl dimethyl ammonium                              | Ethyl phosphate<br>(bis-amine salt)    |
| Dodecylbenzyl trimethyl ammonium                        | Diocetyl phosphate                     |
|                                                         | Dibenzyl phosphate                     |
| Dodecyl dimethyl butyl ammonium                         | Diallyl phosphate                      |
| Benzyl trimethyl ammonium                               | Methyl phenyl phosphate                |
| Allyl tributyl ammonium                                 | Bis(octylphenyl) phosphate             |
| Trimethyl hexadecenyl ammonium<br>(Unsaturated R Group) | Di-n-dodecyl phosphate                 |
| Heptadecyl trimethyl ammonium                           | Diethyl dithiophosphate                |
| Triocetyl methyl ammonium                               | Di-n-butyl-dithiophosphate             |
| Nonyl trimethyl ammonium                                | Dibenzyl dithiophosphate               |
| Tris(n-tridecyl) methyl ammonium                        | Diphenyl dithiophosphate               |
| Tris(n-dodecyl) methyl ammonium                         | Bis(nonyl phenyl) phosphate            |
| Tris(isooctyl) methyl ammonium                          | Butyl phosphate                        |
| Dimethyl butyl hexadecyl ammonium                       | Methyl octylphosphonate                |
| Triethyl methyl ammonium                                | Hexadecyl phosphonate                  |
| 2-ethylhexyl dimethyl dodecyl ammonium                  | Methyl hexadecyl phosphonate           |
| Dimethyl ethyl dodecyl ammonium                         | Methyl tertiary-butyl phosphonate      |
| Dimethyl butyl dodecyl ammonium                         | Methyl carbomethoxy-methyl phosphonate |
| Trimethyl dodecyl ammonium                              |                                        |

-continued

| Ammonium Ions                                                                         | Phosphorus Ester Anions        |
|---------------------------------------------------------------------------------------|--------------------------------|
| Hexadecyl dimethyl ethyl ammonium                                                     |                                |
| Tris(dodecyl) butyl ammonium                                                          |                                |
| Tetramethyl ammonium                                                                  |                                |
| Trimethyl benzyl ammonium                                                             |                                |
| 4-acetyl N-methyl pyridinium                                                          |                                |
|                                                                                       |                                |
| 10  | 1-(N,N-dimethyl)-1-imidazolium |
|                                                                                       | 1-(N,N-dimethyl)-1-pyrazolium  |
| 15 N-methyl oxazolium                                                                 |                                |
| N-butyl quinolinium                                                                   |                                |
| N-methyl pyrrolium                                                                    |                                |
| N,N-diethyl pyrrolidinium                                                             |                                |
| N-methyl,N-hexyl piperidinium                                                         |                                |
| N-methyl,N-butyl piperidinium                                                         |                                |
| N-isopropyl thiazolium                                                                |                                |
| N-ethyl,N-methyl phenothiazinium                                                      |                                |
| 20 N-methyl pyridinium                                                                |                                |

|    |                                                                                                                                                                                                                                         |
|----|-----------------------------------------------------------------------------------------------------------------------------------------------------------------------------------------------------------------------------------------|
| 25 | Members of the ammonium ions can be combined with members of the phosphorus ester anions to generate typical compounds which can be used in this invention. For example, particularly preferred ammonium salts of phosphorus acids are: |
|    | Hexadecyl trimethyl ammonium diphenyl phosphate                                                                                                                                                                                         |
|    | Decyl trimethyl ammonium diphenyl phosphate                                                                                                                                                                                             |
| 30 | Didodecyl dimethyl ammonium diphenyl phosphate                                                                                                                                                                                          |
|    | Dimethyl propyl dodecyl ammonium diphenyl phosphate                                                                                                                                                                                     |
|    | Dodecylbenzyl trimethyl ammonium diphenyl phosphate                                                                                                                                                                                     |
| 35 | Allyl tributyl ammonium diphenyl phosphate                                                                                                                                                                                              |
|    | Trimethyl hexadecenyl ammonium diphenyl phosphate                                                                                                                                                                                       |
|    | Bis(dodecyl trimethyl ammonium)phenyl phosphate                                                                                                                                                                                         |
|    | Bis(octadecyl trimethyl ammonium)phenyl phosphate                                                                                                                                                                                       |
|    | Decyl trimethyl ammonium dimethyl phosphate                                                                                                                                                                                             |
| 40 | Didodecyl dimethyl ammonium methyl methylphosphonate                                                                                                                                                                                    |
|    | Bis(didodecyl dimethyl ammonium)methylphosphonate                                                                                                                                                                                       |
|    | dodecyl trimethyl ammonium dimethyl phosphate                                                                                                                                                                                           |
|    | Dodecyl trimethyl ammonium dibenzyl phosphate                                                                                                                                                                                           |
| 45 | Dodecyl trimethyl ammonium methyl phenyl phosphate                                                                                                                                                                                      |
|    | Dodecyl trimethyl ammonium bis(nonylphenyl)phosphate                                                                                                                                                                                    |
|    | Dodecyl trimethyl ammonium diphenyl dithiophosphate                                                                                                                                                                                     |
| 50 | Octadecyl trimethyl ammonium diphenyl dithiophosphate                                                                                                                                                                                   |
|    | Dodecyl trimethyl ammonium diethyl dithiophosphate                                                                                                                                                                                      |
|    | Dodecyl trimethyl ammonium diallyl phosphate                                                                                                                                                                                            |
| 55 | Dodecyl trimethyl ammonium diphenyl phosphate                                                                                                                                                                                           |
|    | Didodecyl dimethyl ammonium di-n-dodecyl phosphate                                                                                                                                                                                      |
|    | Dodecyl trimethyl ammonium di-n-dodecyl phosphate                                                                                                                                                                                       |
|    | Benzyl trimethyl ammonium methyl phenyl phosphate                                                                                                                                                                                       |
| 60 | Trimethyl hexadecenyl ammonium methyl phenyl phosphate                                                                                                                                                                                  |
|    | Octadecyl trimethyl ammonium diphenyl phosphate                                                                                                                                                                                         |
|    | Tridecyl trimethyl ammonium diphenyl phosphate                                                                                                                                                                                          |
|    | Heptadecyl trimethyl ammonium diphenyl phosphate                                                                                                                                                                                        |
| 65 | Benzyl trimethyl ammonium dibenzyl dithiophosphate                                                                                                                                                                                      |
|    | Hexadecyl trimethyl ammonium dimethyl phosphate                                                                                                                                                                                         |
|    | Triocetyl methyl ammonium diphenyl phosphate                                                                                                                                                                                            |
|    | Heptadecyl trimethyl ammonium dimethyl phosphate                                                                                                                                                                                        |

Tris(n-tridecyl)methyl ammonium diphenyl phosphate  
 Tris(n-dodecyl)methyl ammonium diphenyl phosphate  
 Tris(isooctyl)methyl ammonium diphenyl phosphate  
 Dimethyl butyl hexadecyl ammonium dibutyl phosphate  
 Triethyl methyl ammonium methyl methylphosphonate  
 N-methyl, N-butyl piperidinium dibutyl phosphate  
 2-ethylhexyl dimethyl dodecyl ammonium diphenyl phosphate  
 Dimethyl ethyl dodecyl ammonium diethyl phosphate  
 Dimethyl butyl dodecyl ammonium dibutyl phosphate  
 Trimethyl dodecyl ammonium methyl methylphosphonate  
 Hexadecyl dimethyl ethyl ammonium diethyl phosphate  
 Tris(dodecyl)butyl ammonium dibutyl phosphate  
 Tetramethyl ammonium methyl octylphosphonate  
 Trimethyl benzyl ammonium methyl octylphosphonate  
 Tetramethyl ammonium methyl hexadecylphosphonate  
 20 Benzyl trimethyl ammonium methyl hexadecylphosphonate  
 Tetramethyl ammonium methyl tertiary-butyl-phosphonate  
 Benzyl trimethyl ammonium methyl tertiary-butyl-phosphonate  
 Tetramethyl ammonium methyl carbomethoxymethylphosphonate  
 Benzyl trimethyl ammonium methyl carbomethoxymethylphosphonate  
 Trimethyl tertiary-octylphenyl ammonium diphenyl phosphate  
 Trimethyl tertiary-octylphenyl ammonium methyl methylphosphonate  
 Trimethyl tertiary-octylphenyl ammonium bis(nonylphenyl)phosphate  
 30 Tetramethyl ammonium bis(nonylphenyl)phosphate  
 Benzyltrimethyl ammonium bis(nonylphenyl) phosphate



The quaternary ammonium salts of diesters of phosphoric acid which contain no N-H bonds can be prepared by known means as outlined in British Pat. No. 1,199,015 (1970) and in the preprints of the Symposium

on Deposit, Wear, and Emission Control by Lubricants and Fuel Additives presented in the Division of Petroleum Chemistry of the American Chemical Society, N.Y. City Meeting, Sept. 7-12, 1969, page A-110. These methods include:

1. Reaction of an amine with a triester of phosphoric acid in which the triester alkylates the amine. These reactions usually take place above 40°-60° and can be run neat or in alcohol solvents. All volatile species are then removed by distillation to leave behind the phosphoric acid diester salt of a quaternary ammonium cation.



15 where R, R<sup>1</sup> and R<sup>2</sup> can be the same or different and wherein R and R<sup>1</sup> can be conjoint and can contain one or more heterocyclic atoms, such as oxygen, nitrogen, and mixtures thereof; and represent alkyl, aralkyl, and alkenyl groups. R<sup>3</sup> is preferably of the benzyl, allyl or lower alkyl (especially methyl) type, R<sup>4</sup> can be alkyl, aryl, alkaryl, alkoxy, aryloxy, alkaryloxy, alkyloxy, and also substituted alkyl, such as carboalkoxy, carboalkoxyalkyl, carboalkoxyaryl and the like.

20 These reactions are well known in the art. Reactions of primary aromatic amines are discussed in Thomas et al, Journal of the American Chemical Society, Volume 68, at page 895 (1946). Reactions of secondary and tertiary amines are discussed in Clark et al, Journal of the Chemical Society, page 2023 (1950); Atherton et al, ibid, page 1106, (1948) and Baddiley et al, ibid, page 815 (1949). Reactions of mixed aryl alkyl phosphate esters with pyridine are discussed in Osborne, Journal of Organic Chemistry, Volume 29, page 3570 (1964); See also Kirby et al, Organic Chemistry of Phosphorus, page 209 ff., (Elsevier 1967). For reactions of phosphoric acid triesters, see Kosolapoff et al, Organic Phosphorus Compounds, Volume 6, at pages 236, 515 and 523-526 (Wiley-Interscience, 1973). For reactions of phosphonates with nucleophiles, see Hudson, Structure and Mechanism in Organophosphorus Chemistry, pg. 110 (Academic Press 1965).

25 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 98

present in the fluid, or by significantly increasing the conductivity of the fluid.

Both approaches have been explored with some degree of success. This is surprising due to the fact that eliminating ionic impurities actually lowers the conductivity. This appears to indicate two contradictory approaches to the problem of ameliorating damage caused by erosion. Recent experiments have shown that the elimination of ionic impurities by filtration through an activated clay will control erosion caused by a phosphate ester hydraulic fluid. However, this is not a practical solution since erosion begins again soon after the filtration is discontinued. In addition, filtration on aircraft is virtually impossible.

The addition of ammonium salts of phosphorus acids to various base stocks has been found to effectively inhibit damage. Furthermore, conductivity measurements of these fluids containing ammonium salts of phosphorus acids indicated increased conductivity. It is too early to conclusively attribute conductivity as an explanation of the mechanism, or for evaluating the effectiveness of damage inhibitors. However, conductivity does serve as some indicia, although further research in this area is deemed necessary and desirable.

Typical conductivities of commercial phosphate ester aircraft hydraulic fluids on the market today vary from about 0.02 to about 6 micromhos/centimeter.

Functional fluid compositions to which the ammonium salt of phosphorus acid compositions can be added are referred to as base stocks. They include, but are not limited to esters and amides of phosphorus acids, mineral oil and synthetic hydrocarbon oil base stocks, hydrocarbyl silicates, silicones, aromatic ether and thioether compounds, chlorinated biphenyl, monoesters, dicarboxylic acid esters, esters of polyhydric compounds, polyalkylene ether glycols and alcohols as well as their esters.

The concentration of ammonium salts of phosphorus acids in the functional fluid is adjusted in terms of the particular system and the functional fluid to inhibit and control damage. Thus, it has been found that the additive response, that is, the concentration of an ammonium salt of phosphorus acid required to inhibit and control damage of a base stock varies according to the base stock or blends of base stocks employed.

Thus, for the base stocks useful in the practice of this invention the concentration of ammonium salts of phosphorus acid is from about 0.01 percent to about 15 percent by weight, the particular concentration being that amount which will effectively inhibit and control damage. The preferred additive concentration is from about 0.025 to about 5 weight percent, more preferably, from about 0.1 to about 0.5 weight percent. Therefore, included within the present invention are compositions comprising a functional fluid and a damage-inhibiting amount of an ammonium salt of phosphorus acids, that is, the ammonium salt is added, in a concentration sufficient to control and inhibit damage. The functional fluid compositions of this invention can be compounded in any manner known to those skilled in the art for the incorporation of an additive into a base stock and preferably, by adding an ammonium salt of phosphorus acids to the base stock with stirring until a fluid composition is obtained.

As indicated above, the compositions of this invention can employ a wide variety of base stocks. Particularly, suitable base stock materials are the esters and

amides of an acid of phosphorus represented by the structure:



wherein Y is selected from the group consisting of oxygen, sulfur and



Y<sub>1</sub> is selected from the group consisting of oxygen, sulfur and



and Y<sub>2</sub> is selected from the group consisting of oxygen, sulfur and



R, R<sub>1</sub>, R<sub>2</sub>, R<sub>3</sub>, R<sub>4</sub> and R<sub>5</sub> are each selected from the group consisting of alkyl, alkoxy, aryl, substituted aryl and substituted alkyl wherein R, R<sub>1</sub>, R<sub>2</sub>, R<sub>3</sub>, R<sub>4</sub> and R<sub>5</sub> each can be identical or different with respect to any other radical, and a, b and c are whole numbers having a value of 0 to 1 and the sum of a+b+c is from 1 to 3.

Generally, the number of carbon atoms in the alkyl groups will vary from 1 to 30. Included within the alkyl groups are the cycloalkyls and alkyl substituted cycloalkyls. Typical examples of alkyl radicals are as follows:

methyl, ethyl, normal propyl, isopropyl, normal butyl, isobutyl, secondary butyl, tertiary butyl, normal amyl, isoamyl, 2-methylbutyl, 2,2-dimethyl propyl, 1-methyl butyl, diethylmethyl, 1,2-dimethyl propyl, tertiary amyl, normal hexyl, 1-methylamyl, 1-ethyl butyl, 1,2,2-trimethyl propyl, 3,3-dimethyl butyl, 1,1,2-trimethyl propyl, 2-methyl amyl, 1,1-dimethyl butyl, 1-ethyl 2-methyl propyl, 1,3-dimethyl butyl, isohexyl, 3-methylamyl, 1,2-dimethyl butyl, 1-methyl 1-ethyl propyl, 2-ethyl butyl, normal heptyl, 1,1,2,3-tetramethyl propyl, 1,2-dimethyl 1-ethyl propyl, 1,1,2-trimethyl butyl, 1-isopropyl 2-methyl propyl, 1-methyl 2-ethyl butyl, 1,1-diethyl propyl, 2-methyl hexyl, 1,1-dimethyl amyl, 1-isopropyl butyl, 1-ethyl 3-methyl butyl, 1,4-dimethyl amyl, isoheptyl, 1-methyl 1-ethyl butyl, 1-ethyl 2-methyl butyl, 1-methyl hexyl, 1-propyl butyl, normal octyl, 1-methyl heptyl, 1,1-diethyl 2-methyl propyl, 1,1,3,3-tetramethyl butyl, 1,1-diethyl butyl, 1,1-dimethyl hexyl, 1-methyl 1-ethyl amyl, 1-methyl 1-propyl butyl, 2-ethyl hexyl, 6-methyl heptyl (iso-octyl), normal nonyl, 1-methyl octyl, 1-ethyl heptyl, 1,1-dimethyl heptyl, 1-ethyl 1-propyl butyl, 1,1-diethyl 3-methyl butyl, diisobutyl methyl, 3,5,5-trimethyl hexyl, 3,5-dimethyl heptyl, normal decyl, 1-propyl heptyl, 1,1-diethyl hexyl, 1,1-dipropyl butyl, 2-isopropyl 5-methyl hexyl and C<sub>11</sub>-C<sub>18</sub> alkyl groups such as dodecyl, tridecyl, hexadecyl and the like. Also included are aralkyl groups, e.g., benzyl, alpha- or beta-phenylethyl,

alpha-alpha dimethyl benzyl and the like, with the alkyl portion having from 1 to 30 carbon atoms. Also included are cyclobutyl, cyclohexyl, cycloheptyl and the like. Also included are alkaryl groups such as methyl-phenyl, ethylphenyl and the like. Also included are 5 alkoxy alkyl such as methoxy ethyl, ethoxy ethyl, butoxyethyl, butoxy butyl and the like.

Typical examples of substituted alkyl radicals are the haloalkyl radicals which can be represented by the structure: 10



where Hal refers to a halogen, m is less than or equal to 2n+1 and n may have any value from 0 to 18, and R<sub>6</sub> and R<sub>7</sub> can be hydrogen, halogen such as F, Cl, Br and 20 I, or alkyl radicals. Preferred radicals are those where Hal is fluoro and include those represented by the following formulas:



-continued



30 where R<sub>6</sub> and R<sub>7</sub> have their aforescribed significance. The halogenated alkyl radicals can be primary, secondary or tertiary.

35 Other suitable fluorine-containing radicals include fluorinated alkoxyalkyl radicals particularly those represented by the following formulas:



where  $R_6$  and  $R_7$  have their aforescribed significance.

It is also contemplated within the scope of this invention that the hydrogen and the fluorine in the previously described haloalkyl radicals can be replaced by other halogens, such as chlorine or bromine.

Typical examples of aryl and substituted aryl radicals are phenyl, cresyl, xylyl, halogenated phenyl, alkoxy-alkyl phenyl, cresyl and xylyl in which the available hydrogen on the aryl or substituted aryl is partially or totally replaced by a halogen, o-, m- and p-trifluoromethylphenyl, o-, m- and p-2,2,2-trifluoroethylphenyl, o-, m- and p-3,3,3-trifluoropropylphenyl and o-, m-, and p-4,4,4-trifluorobutylphenyl. Also included are isopropylphenyl, butylphenyl, alpha-alkylbenzylphenyl and alpha,alpha-dialkylbenzylphenyl, e.g. alpha-methylbenzylphenyl, alpha,alpha dimethylbenzylphenyl.

The orthosilicates useful as base stocks include the tetraalkyl orthosilicates such as tetra(octyl)orthosilicates, tetra(2-ethylhexyl)orthosilicates and the tetra(isooctyl) orthosilicates and those in which the isooctyl radicals are obtained from isooctyl alcohol which is derived from the oxo process, and the (trialkoxy silico)-trialkyl orthosilicates, otherwise referred to as hexa(alkoxy) disiloxanes, such as hexa(2-ethylbutoxy) disiloxane and hexa(2-ethylhexoxy) disiloxane.

The preferred tetraalkyl orthosilicates and hexa(alkoxy) disiloxanes are those in which the alkyl or alkoxy radicals have from 4 to 12 carbon atoms and in which the total number of carbon atoms in the orthosilicate is from 16 to 60.

In addition to the hexa(alkoxy) disiloxanes referred to above, other hexa(alkoxy) disiloxanes can be used in which the aliphatic radical of the alkoxy groups are for example, 1-ethylpropyl, 1,3-dimethylbutyl, 2-methylpentyl, 1-methylhexyl, 1-ethylpentyl, 2-butylhexyl and 1-methyl-4-ethyloctyl.

The orthosilicates and alkoxy polysiloxanes can be represented by the general structure:



wherein  $R_8$ ,  $R_9$  and  $R_{10}$  each can be alkyl, substituted alkyl, aryl, substituted aryl and can be identical or different with respect to any other radical, O is oxygen, Si is silicon, X is a member of the group consisting of carbon and silicon, m is a whole number having a value of 0 or 1, n is an integer having a value of from 1 to about 200 or more and when X is carbon, m is 0, n is 1 and  $R_{11}$ ,  $R_{12}$  and  $R_{13}$  each can be hydrogen, alkyl, substituted alkyl, aryl and substituted aryl radicals and when X is silicon m is 1, n is an integer having a value of from 1 to about 200 or more and  $R_{11}$ ,  $R_{12}$  and  $R_{13}$  each can be alkyl, substituted alkyl, aryl and substituted aryl.

Typical examples of substituted aryl radicals are o-, m- and p-chlorophenyl, o-, m- and p-bromophenyl, o-, m- and p-fluorophenyl, alpha,alpha,alpha-trichlorocresyl, alpha,alpha,alpha-trifluorocresyl, xylyl and o-, m- and p-cresyl. Typical examples of alkyl and haloalkyl radicals are those heretofore described.

The siloxanes or silicones useful as base stocks are represented by the general structure:



wherein  $R_{14}$ ,  $R_{15}$ ,  $R_{16}$ ,  $R_{17}$ ,  $R_{18}$  and  $R_{19}$  can each be alkyl, substituted alkyl, aryl and substituted aryl radicals and n is a whole number from about 0 to about 2000 or more. Typical examples of alkyl and haloalkyl radicals along with the number of carbon atoms are those heretofore described. Typical examples of the siloxanes are poly(methyl) siloxane, poly(methyl, phenyl) siloxane, poly(methyl, chlorophenyl) siloxane and poly(methyl, 3,3,3-trifluoropropyl) siloxane.

Typical examples of substituted aryl radicals and o-, m- and p-chlorophenyl, o-, m- and p-bromophenyl, o-, m- and p-fluorophenyl, alpha,alpha,alpha-trichlorocresyl, alpha, alpha, alpha-trifluorocresyl, o-, m- and p-cresyl and xylyl.

Dicarboxylic acid esters which are suitable as base stocks are represented by the structure:



wherein  $R_{20}$  and  $R_{22}$  are each selected from the group consisting of alkyl, substituted alkyl, aryl and substituted aryl and  $R_{21}$  is a divalent radical selected from the group consisting of alkylene and substituted alkylene, and are prepared by esterifying dicarboxylic acids such as adipic acid, azelaic acid, suberic acid, sebacic acid, hydroxysuccinic acid, fumaric acid, maleic acid, etc., with alcohols such as butyl alcohol, hexyl alcohol, 2-ethylhexyl alcohol, dodecyl alcohol, 2,2-dimethyl heptanol, 1-methyl cyclohexyl methanol, and the like.

Typical examples of alkyl, aryl substituted alkyl and substituted aryl radicals are given above.

Polyesters which are suitable as base stocks are represented by the structure:



wherein  $R_{23}$  is selected from the group consisting of hydrogen and alkyl,  $R_{24}$  and  $R_{25}$  are each selected from the group consisting of alkyl, substituted alkyl, aryl and substituted aryl, a is a whole number having a value of 0 to 1, Z is a whole number having a value of 1 to 2 and when Z is 1,  $R_{26}$  is selected from the group consisting of hydrogen, alkyl acyloxy and substituted acyloxy and when Z is 2,  $R_{26}$  is oxygen, and are prepared by esterifying such polyalcohols as pentaerythritol, dipentaerythritol, trimethylolpropane, trimethylethane and neo-

pentyl glycol with such acids as propionic, butyric, isobutyric, n-valeric, capric, caproic, n-heptylic, caprylic, 2-ethylhexanoic, 2,2-dimethylheptanoic and pelargonic. Typical examples of alkyl, substituted alkyl, aryl and substituted aryl radicals are given above.

Other esters which are also suitable as base stocks are the mono esters.

Another class of compositions which are suitable as base stocks for this invention are the polyphenyl ethers, polyphenyl thioethers, or mixtures thereof, as represented by the structure:



wherein A, A<sub>1</sub>, A<sub>2</sub>, and A<sub>3</sub> are each a chalcogen having an atomic number of 8 to 16, X, X<sub>1</sub>, X<sub>2</sub>, X<sub>3</sub> and X<sub>4</sub> each are selected from the group consisting of hydrogen, alkyl, haloalkyl, halogen, arylalkyl and substituted arylalkyl, m, n and o are whole numbers, each having a value of 0 to 8 and a is a whole number having a value of 0 to 1 provided that when a is 0, n can have a value of 1 to 2. Typical examples of alkyl and substituted alkyl radicals are given above. Typical examples of such base stocks are 2- to 7-ring ortho-, meta- and para-polyphenyl ethers and mixtures thereof, 2- to 7-ring ortho-, meta-, and para-polyphenyl thioethers and mixtures thereof, mixed polyphenyl ether-thioether compounds in which at least one of the chalcogens represented by A, A<sub>1</sub>, A<sub>2</sub> and A<sub>3</sub> is dissimilar with respect to any one of the other chalcogens, dihalogenated diphenyl ethers, such as 4-bromo-3'-chlorodiphenyl ethers and bis-phenoxy biphenyl compounds and mixtures thereof.

Hydrocarbon oils including mineral oils derived from petroleum sources and synthetic hydrocarbon oils are suitable base stocks. The physical characteristics of functional fluids derived from a mineral oil are selected on the basis of the requirements of the fluid system and therefore this invention includes as base stocks mineral oils having a wide range of viscosities and volatilities such as naphthenic base, paraffinic base and mixed base mineral oils.

The synthetic hydrocarbon oils include but are not limited to those oils derived from oligomerization of olefins such as polybutenes and oils derived from high or alpha-olefins of from 4 to 20 carbon atoms such as by acid catalyzed dimerization and then oligomerization using mixtures of aluminum alkyls and titanium halides as catalysts, or Friedel-Crafts catalysts, or peroxide catalysts.

Chlorinated biphenyls and terphenyls are also useful as base stocks.

The fluid compositions of this invention when utilized as a functional fluid can also contain acid acceptors, dyes, pour point depressants, thickeners, antioxidants, antifoam agents, viscosity index improvers such as polyalkyl acrylates, polyalkyl methacrylates, polycyclic polymers polyurethanes, polyalkylene oxides and polyesters, lubricity agents, water and the like.

It is also contemplated that the base stocks as aforementioned can be utilized singly or as a blend containing two or more base stocks in varying proportions.

Most often, the base stock material will contain esters and/or amides of an acid of phosphorus, and blends of the aforesaid with one or more of the following materials: mineral oils, synthetic hydrocarbon oils, orthosilicates, alkoxypolysiloxanes, silicones, polyphenyl ethers, polyphenyl thioethers, chlorinated biphenyls, esters of dicarboxylic acids and monohydric alcohols, esters of monocarboxylic acids and monohydric alcohols, esters of monocarboxylic acids and polyhydric alcohols, polyalkylene ether alcohols and esters thereof, and blends thereof. The base stocks can also contain other fluids which include, in addition to the functional fluids, desired fluids derived from coal tar products, synthetics, and synthetic oils, e.g., alkylene polymers (such as polymers of propylene, butylene, etc., and mixtures thereof), alkylene oxide type polymers (e.g., propylene oxide polymers), and derivatives, including alkylene oxide polymers prepared by polymerizing the alkylene oxide in the presence of water or alcohol, e.g., ethyl alcohol, alkyl benzenes, (e.g., monoalkyl benzene such as dodecyl benzene, tetradecyl benzene, etc.) and dialkyl benzene (e.g., n-nonyl 2-ethyl hexyl benzene); polyphenyls, (e.g., biphenyls and terphenyls), halogenated benzene, halogenated lower alkyl benzene and monohalogenated diphenyl ethers.

In the preferred form of the present invention, the ammonium salt of phosphorus acid composition of the present invention is combined with a phosphate ester functional fluid base stock. The base stock will consist primarily of trialkylphosphates being present in amounts from 50 to 95% by weight and preferably from 60 to 90% by weight. The trialkylphosphates which give optimum results are those wherein each of the alkyl groups contain from 1 to 20 carbon atoms, preferably from 3 to 12 carbon atoms and more preferably, from 4 to 9 carbon atoms. The alkyl groups are preferably of straight chain configuration. A single trialkyl phosphate can contain the alkyl group in all three positions or can possess a mixture of different alkyl groups. Mixtures of various trialkyl phosphates can be used. Suitable species of trialkyl phosphates which can be employed as the base stock composition include tripropyl phosphates, tributyl phosphates, trihexyl phosphates, trioctyl phosphates, dipropyl octyl phosphates, dibutyl octyl phosphates, dipropyl hexyl phosphate, dihexyl octyl phosphate, dihexyl propyl phosphate, and propyl butyl octyl phosphate.

The trialkyl phosphates can be combined with triaryl phosphates or mixed alkyl aryl phosphates. Preferred triaryl phosphates are tricresyl phosphate, cresyl diphenyl phosphate, trixylenyl phosphate, tertiary-butylphenyl phenyl phosphates, ethylphenyl diresyl phosphate or isopropylphenyl diphenyl phosphate, phenyl-bis(4-alpha-methylbenzylphenyl) phosphate, diphenyl decyl phosphate, diphenyl octyl phosphate, methyl diphenyl phosphate, butyl diresyl phosphate and the like. In one preferred embodiment, a base stock containing primarily trixylenyl phosphate is employed. The triaryl phosphates function as a thickener for the trialkyl phosphates. Thus, the amount of triaryl phosphate may range between 0 to 35% by weight. The preferred range of the triaryl phosphates will be from about 5 to about 30% by weight of the composition.

Conventional polymeric thickeners or viscosity index (VI) improvers can be blended with the mixture of

trialkyl and triaryl phosphate material to achieve the desired viscosity. Typical thickeners used can be polyacrylates, polymethacrylates, polyethylene oxides, polypropylene oxides, polyesters, and the like.

Preferably, a polyester based upon an azelaic acid and a diol such as propylene glycol, and the like, in the range of 0.3 to 20% by weight is used as the thickener.

Combinations of antioxidants and/or acid acceptors in amounts ranging from about 0.1 to about 5% by weight can also be incorporated into the functional fluid composition, such as, epoxides and/or amines. The combination of 3,4-epoxycyclohexylmethyl 3,4-epoxycyclohexane carboxylate and phenyl-alphanaphthylamine has been found to be very effective.

Corrosion inhibitors such as benzotriazole, quinizarin or the like in an amount ranging between 0.001 and 0.5% by weight can be added to the mixture and thoroughly blended therewith. A dye in a concentration range between 5 and 20 parts per million can be added to the composition and blended therewith in a conventional manner. Effective amounts of a silicone anti-foaming agent can also be incorporated into the composition and are usually most effective in an amount ranging between 5 and 50 parts per million.

The functional fluids of this invention can contain up to about 1% by weight of water. It is preferred, however, to maintain water levels below 0.6 weight percent, and most preferably below about 0.3 weight percent.

The invention can be illustrated by the following non-limiting examples.

In the examples and throughout the specification, all parts and percentages are by weight, unless otherwise noted.

#### EXAMPLE 1

A base stock consisting of 78.98 weight percent of tributyl phosphate and 9.70 weight percent of mixed 40 cresyl and xylenyl phosphates with a viscosity of approximately 220 Saybolt Universal Seconds at 100° F. is combined with 9.00 weight percent of a polyester thickener, Plastolein® 9789 sold by Energy Industries. Thereafter, 1.0 weight percent of 3,4-epoxycyclohexylmethyl 3,4-epoxycyclohexane carboxylate and 1.0 weight percent of phenyl alpha-naphthylamine are blended into this mixture. Then 0.02 weight percent of benzotriazole is thoroughly blended therewith along with conventional dye and antifoam agent in the amount of 20 parts per million, and 15 parts per million, respectively. Thereafter, dodecyl trimethyl ammonium diphenyl phosphate is blended into the mixture at various addition levels including 0.1% and 0.3% by weight.

The composition prepared as above was tested in an apparatus consisting of a Boeing 737 trailing edge flap valve pressurized by a Vickers axial piston pump together with related equipment required to assure that the apparatus will operate according to the requirements of Section 10.2 of SAE specification AS 1241 pertaining to the erosion resistance of fire resistant aircraft hydraulic fluids. Fluids are evaluated on the basis of leakage rate increase for the valve when it is in the closed or null position. The results of the dodecyl trimethyl ammonium diphenyl phosphate addition into the phosphate ester fluid are as follows:

| % BY WEIGHT OF DODECYL TRIMETHYL AMMONIUM DIPHENYL PHOSPHATE | LEAKAGE RATE INCREASE (cc/min/hr.) | CONDUCTIVITY (micromhos/cm) |
|--------------------------------------------------------------|------------------------------------|-----------------------------|
| None                                                         | 7.0                                | 0.021                       |
| 0.1                                                          | 2.0                                | 0.10                        |
| 0.3                                                          | 0.0                                | 0.29                        |

The test results show that the addition of an effective amount of dodecyl trimethyl ammonium diphenyl phosphate to a phosphate ester hydraulic fluid inhibits damage to hydraulic systems.

#### EXAMPLE 2

A similar erosion test was performed on the phosphate ester fluid described in Example 1 with 0.3% by weight of dodecyl trimethyl ammonium diphenyl phosphate. In this test the concentration of chlorinated solvents was gradually increased up to a final level of 2000 parts per million (PPM) of chlorine.

| Total Chlorine (PPM)                                                         | Total Test Time (Hrs.) | Leakage Rate Increase(cc/min/hr) |
|------------------------------------------------------------------------------|------------------------|----------------------------------|
| 40 (base level)                                                              | 440                    | 0                                |
| 275 (as $\text{CH}_3\text{CCl}_3$ )                                          | 625                    | 0                                |
| 444 (as $\text{CH}_3\text{CCl}_3$ )                                          | 730                    | 0                                |
| 938 (as $\text{CH}_3\text{CCl}_3$ )                                          | 830                    | 0                                |
| 2000 (as $\text{CH}_3\text{CCl}_3$ and $\text{CF}_2\text{ClCCl}_2\text{F}$ ) | 910                    | 0                                |

This data has been plotted in the FIGURE and illustrates the utility of dodecyl trimethyl ammonium diphenyl phosphate for preventing damage caused to hydraulic systems by chlorine contaminated phosphate ester hydraulic fluids.

#### EXAMPLE 3

An erosion test was performed on a Boeing Material Spec. 311C (BMS 311-C) qualified phosphate ester aircraft hydraulic fluid contaminated with 1000 PPM of chlorine as 1,1,1-trichloroethane. After the erosion rate was established, the phosphate ester fluid described in Example 1 with 0.3% by weight of dodecyl trimethyl ammonium diphenyl phosphate was added in increments to the contaminated fluid. The following data was obtained in this test:

| QUALIFIED BMS 311-C PHOSPHATE ESTER HYDRAULIC FLUID + 1000 PPM CHLORINE AS $\text{CH}_3\text{CCl}_3$         |                                   |
|--------------------------------------------------------------------------------------------------------------|-----------------------------------|
| Total Wt. % of Phosphate Ester Fluid Containing 0.3% by Wt. of Dodecyl Trimethyl Ammonium Diphenyl Phosphate | Leakage Rate Increase (cc/min/hr) |
| None                                                                                                         | 6.0                               |
| 20                                                                                                           | 6.0                               |
| 35                                                                                                           | 0.8                               |
| 50                                                                                                           | 0                                 |

The above results illustrate the utility of a formulation containing dodecyl trimethyl ammonium diphenyl phosphate for arresting the damage caused to hydraulic systems by chlorine contaminated phosphate ester hydraulic fluids.

#### EXAMPLE 4

A blend similar to that described in Example 1 was prepared. Two formulations were prepared with this

blend. The first contained 0.2 weight percent of dodecyl trimethyl ammonium diphenyl phosphate and the sec-

triaryl and trialkyl phosphates. The results of these tests are tabulated below:

| Additive                                                                           | Percent By Weight | Leakage Rate Increase (cc/min./hr.) |
|------------------------------------------------------------------------------------|-------------------|-------------------------------------|
| None                                                                               | None              | +22                                 |
| Dodecyl trimethyl ammonium methyl methyl phosphonate                               | 0.3               | +1.2                                |
| Hexadecyl ethyl dimethyl ammonium diethyl phosphate                                | 0.5               | -0.8                                |
| Benzyl trimethyl ammonium diphenyl phosphate                                       | 0.3               | +0.3                                |
| Benzyl trimethyl ammonium bis-nonyl-phenyl phosphate                               | 0.3               | +0.3                                |
| Benzyl phenylethyl dimethyl ammonium bis-phenylethyl phosphate                     | 0.3               | -0.8                                |
|  | 0.3               | -0.8                                |
|  | 0.3               | +1.6                                |

ond contained 0.2 weight percent of trioctyl methyl phosphonium dimethyl phosphate. These formulations were subjected to stability tests described in Boeing <sup>30</sup> Material Specification 311-C. The following results were obtained in these tests:

#### Boeing Thermal Stability Test

Test Conditions: 250° F., 168 hours duration, steel, magnesium, cadmium plated steel, copper, and aluminum present as catalysts.

| Fluid                       | Viscosity Change (cs) |         | Acid No. Increase (mgKOH/g) |
|-----------------------------|-----------------------|---------|-----------------------------|
|                             | 100° F.               | 210° F. |                             |
| Base Blend + 0.2 Weight     |                       |         |                             |
| Percent Dodecyl Trimethyl   |                       |         |                             |
| Ammonium Diphenyl Phosphate | +0.10                 | +0.03   | 0                           |
| Base Blend + 0.2 Weight     |                       |         |                             |
| Percent Trioctyl Methyl     |                       |         |                             |
| Phosphonium Dimethyl        |                       |         |                             |
| Phosphate                   | -1.11                 | -0.42   | 1.2                         |
| BMS 311-C Specification     |                       |         |                             |
| Limits                      | ±1.0                  | ±0.3    | +0.5                        |

These tests demonstrate that formulations prepared with dodecyl trimethyl ammonium diphenyl phosphate as an additive exhibit greater thermal and oxidative stability than formulations prepared with trioctyl methyl phosphonium dimethylphosphate.

#### EXAMPLE 5

The following compositions were tested in an apparatus consisting of a Boeing 737 trailing edge flap valve pressurized by a Vickers' axial piston pump, together with related equipment required to assure that the apparatus will operate according to the requirements of Section 10.2 of SAE Specification AS 1241 pertaining to the erosion resistance of fire resistant aircraft hydraulic fluids. Fluids were evaluated on the basis of leakage rate increase for the valve when it was in the null or closed position. The base fluid utilized for this test was Stauffer's Aerosafe TM 2300W, comprising a mixture of

#### EXAMPLE 6 Illustrative Embodiment

In an erosion test conducted in a manner similar to that described in Example 1, a fluid comprised of approximately 50% mixed alkyl substituted phosphate ester, 40% aromatic mineral oil, such as NUSO ® 95, sold by Sun Oil Co., 10% pentaerythritol tetraheptanoate, and 0.2% nonyl trimethyl ammonium dioctyl phosphate will exhibit less metal damage than the same fluid without the ammonium phosphate.

What is claimed is:

1. A functional fluid which comprises:
  - (a) major amount of a base stock material selected from the group consisting of esters of an acid of phosphorus, amides of an acid of phosphorus, mixtures of esters and amides of an acid of phosphorus, and blends of the aforesaid with one or more materials selected from the group consisting of mineral oils, synthetic hydrocarbon oils, orthosilicates, alkoxy polysiloxanes, silicones, polyphenyl ethers, polyphenyl thioethers, chlorinated biphenyls, esters of dicarboxylic acids and monohydric alcohols, esters of monocarboxylic acids and monohydric alcohols, esters of monocarboxylic acids and polyhydric alcohols, polyalkylene ether alcohols and esters thereof, and blends thereof; said esters and amides of an acid of phosphorus having the formula:



wherein Y is selected from the group consisting of oxygen, sulfur, and



$Y_1$  is selected from the group consisting of oxygen, sulfur, and



$Y_2$  is selected from the group consisting of oxygen, sulfur, and



$R$ ,  $R_1$ ,  $R_2$ ,  $R_3$ ,  $R_4$ , and  $R_5$  are each selected from the group consisting of alkyl, alkoxy, aryl, substituted aryl and substituted alkyl; and  $a$ ,  $b$ , and  $c$  are whole numbers having a value of 0 to 1 such that the sum  $a+b+c$  has a value from 1 to 3; and

(b) an effective erosion inhibiting amount of  $N$ -methyl,  $N$ -butyl piperidinium dibutyl phosphate.

2. A functional fluid which comprises: (a) a major amount of base stock material selected from the group consisting of esters of an acid of phosphorus, amides of an acid of phosphorus, mixtures of esters and amides of an acid of phosphorus, and blends of the aforesaid with one or more materials selected from the group consisting of mineral oils, synthetic hydrocarbon oils, orthosilicates, alkoxy siloxanes, silicones, polyphenyl ethers, polyphenyl thioethers, chlorinated biphenyls, esters of dicarboxylic acids and monohydric alcohols, esters of monocarboxylic acids and monohydric alcohols, esters of monocarboxylic acids and polyhydric alcohols, polyalkylene ether alcohols and esters thereof, and blends thereof, wherein said esters and amides of an acid of phosphorus have the formula:



wherein  $Y$  is selected from the group consisting of oxygen, sulfur and



$Y_1$  is selected from the group consisting of oxygen, 60 sulfur and



$Y_2$  is selected from the group consisting of oxygen, sulfur and



5  $R$ ,  $R_1$ ,  $R_2$ ,  $R_3$ ,  $R_4$  and  $R_5$  are selected from the group consisting of alkyl, alkoxy, aryl, substituted aryl and substituted alkyl; and  $a$ ,  $b$  and  $c$  are whole numbers having a value of 0 to 1 such that the sum  $a+b+c$  has a value from 1 to 3; and (b) an effective erosion inhibiting amount of 1,3,5-trimethyl pyridinium diphenyl phosphate.

10 3. In a method for inhibiting damage in an hydraulic environment containing a major amount of a base stock material selected from the group consisting of esters of an acid of phosphorus, amides of an acid of phosphorus, mixtures of esters and amides of an acid of phosphorus, and blends of the aforesaid with one or more materials selected from the group consisting of mineral oils, synthetic hydrocarbon oils, orthosilicates, alkoxy siloxanes, silicones, polyphenyl ethers, polyphenyl thioethers, chlorinated biphenyls, esters of dicarboxylic acids and monohydric alcohols, esters of monocarboxylic acids and polyhydric alcohols, polyalkylene ether alcohols and esters thereof, and blends thereof; the improvement which comprises deploying an effective erosion inhibiting amount of  $N$ -methyl,  $N$ -butyl piperidinium dibutyl phosphate.

15 4. In a method for inhibiting damage in a hydraulic environment containing a major amount of a base stock material selected from the group consisting of esters of an acid of phosphorus, amides of an acid of phosphorus, mixtures of esters and amides of an acid of phosphorus, and blends of the aforesaid with one or more materials selected from the group consisting of mineral oils, synthetic hydrocarbon oils, orthosilicates, alkoxy siloxanes, silicones, polyphenyl ethers, polyphenyl thioethers, chlorinated biphenyls, esters of dicarboxylic acids and monohydric alcohols, esters of monocarboxylic acids and monohydric alcohols, esters of monocarboxylic acids and polyhydric alcohols, polyalkylene ether alcohols and esters thereof, and blends thereof; the improvement which comprises deploying an effect erosion inhibiting amount of 1,3,5-trimethyl pyridinium diphenyl phosphate.

20 5. A method of operating an hydraulic pressure device wherein a displacing force is transmitted to a displaceable member by means of a hydraulic fluid comprising a major amount of base stock material selected from the group consisting of esters of an acid of phosphorus, amides of an acid of phosphorus, mixtures of esters and amides of an acid of phosphorus, mixtures of esters and amides of an acid of phosphorus and blends of the aforesaid with one or more materials selected from the group consisting of mineral oils, synthetic hydrocarbon oils, orthosilicates, alkoxy siloxanes, silicones, polyphenyl ethers, polyphenyl thioethers, chlorinated biphenyls, esters of dicarboxylic acids and monohydric alcohols, esters of monocarboxylic acids and monohydric alcohols, esters of monocarboxylic acids and polyhydric alcohols, polyalkylene ether alcohols and esters thereof, and blends thereof; and (b) an effective erosion inhibiting amount of an ammonium salt of a phosphorus acid consisting of 1,3,5-trimethyl pyridinium diphenyl phosphate.

25 6. The method of claim 5 wherein the salt of a phosphorus acid in part (b) is  $N$ -methyl,  $N$ -butyl piperidinium dibutyl phosphate.

\* \* \* \* \*

UNITED STATES PATENT AND TRADEMARK OFFICE  
CERTIFICATE OF CORRECTION

PATENT NO. : 4,252,662

DATED : February 24, 1981

INVENTOR(S) : Theodore A. Marolewski et al.

It is certified that error appears in the above-identified patent and that said Letters Patent is hereby corrected as shown below:

Column 6, line 60, "R<sub>4</sub>NO<sub>2</sub>OP(O) (OR)<sub>2</sub> + NaCl" should read  
-- R<sub>4</sub>NO<sub>2</sub>OP(O) (OR)<sub>2</sub> + NaCl --.

Column 20, line 65, "METHODD" should read -- METHOD --.

Column 18, line 43, "(a) MAJOR AMOUNT" should read -- (a) A MAJOR AMOUNT --

Column 20, line 42, "EFFECTION" should read -- EFFECTIVE --.

Signed and Sealed this

*Fifth Day of October 1982*

[SEAL]

Attest:

GERALD J. MOSSINGHOFF

Attesting Officer

Commissioner of Patents and Trademarks